

## UNITED STATES PATENT OFFICE

2,430,123

## METHOD OF MAKING INSULATING MATERIAL

Ezekiel J. Jacob, Brooklyn, N. Y.

No Drawing. Application May 1, 1944,  
Serial No. 533,663

1 Claim. (Cl. 154—2.6)

1

My present invention relates to insulating materials and more particularly to electrical insulating materials containing micaceous substances, such as mica scales.

It is an object of my present invention to provide composite micaceous materials and articles having high dielectric strength in one direction and small dielectric strength in another.

It is another object of my present invention to provide mica containing materials and articles of variable thermoconductivity, i. e. materials and articles transferring heat differently in various directions.

It is a further object of my present invention to provide improved micaceous materials and articles made therefrom.

With the above objects in view, my present invention mainly consists of an insulating material comprising a binder base and parallelly oriented flakes of a micaceous substance embedded in this binder base. It is an important characteristic feature of my invention that these mica flakes are very small in size, having a diameter of less than .1".

Actually, I use for the purposes of my present invention waste mica splittings which are too small to be used as insulating material; this waste mica is pulverized by crushing, grinding or otherwise to a fineness of 15 mesh or finer. The single particles of the thus prepared mica powder are still flake-shaped.

I have found that by incorporating such minute mica flakes parallelly oriented into a binder substance, I obtain a composition which has different dielectric strength and different thermoconductivity in different directions. That means that the dielectric strength is substantially higher normal to the direction of orientation of the mica flakes than in the direction of such orientation. Contrary thereto, the thermoconductivity of the composition in the direction of parallel orientation of the mica flakes is substantially greater than in direction normal to the same.

I have found that best results are obtained with my new micaceous material if the same contains at least 30% of a binder material; that means that my new insulating material should not contain more than 70% of minute mica flakes. Only if these proportions are maintained, i. e. if my new material contains 30% or more of binder, it is possible to attain proper parallel orientation of the single mica flakes.

I wish to note that in the description and claim I use the term "mica flakes" for the insulating

2

material incorporated into my new insulating composition; this definition has to be understood broadly and is intended to include also substances designated usually as mica powder, mica splittings or mica scales; this term should also be understood to cover powder, scales, flakes or splittings of other micaceous or mica-like substances, such as various other natural silicates having physical characteristics similar to those of mica.

5 I also wish to stress that I may use the most different organic or inorganic binders for the purposes of my present invention and thus the term "binder" as used in the description and claims is intended to include all binders used for such purposes.

10 The most different insulating articles may be made of my new insulating composition. Thus, for instance, it is well adapted to be used for insulating sheets or plates. In this case, all parallelly oriented mica scales are either parallel or normal or at a certain angle to the faces of the sheets or plates. It is evident that orientation of the mica scales in different directions will produce sheets or plates having entirely different 15 electric and other physical characteristics. Thus, for instance, a sheet in which the mica particles are arranged parallel to the faces of the sheet will have a much greater dielectric strength normal to the sheet than a sheet in which the particles 20 extend normal to these faces. Contrary thereto, the thermoconductivity normal to the faces will be much greater in case the scales are arranged 25 normal to these faces than if they are parallel 30 thereto.

35 To produce an insulating composition having parallelly oriented minute mica scales embedded therein is rather difficult. I have found that the difficulties of producing such a composition are best overcome by parallelly orienting the scales 40 of the micaceous substance while they are embedded in a binder base which is in such state as to enable movement of the scales in the binder base. For this purpose, it is preferable to use the binder base in liquid or semi-liquid state.

45 I have furthermore found that it is of great importance that the influence which is exerted in order to parallelly orient the mica flakes is continued while the binder is hardening. If this is not done, the mica particles in the liquid or 50 semi-liquid binder would lose their parallel orientation.

Various methods can be used in order to obtain parallel orientation of the mica flakes:

Thus it is for instance possible to first 55 prepare a mixture of a semi-liquid binder base and

minute mica flakes embedded therein and then to expose this mixture to an electrostatic field under the influence of which the mica flakes will be parallelly oriented in the binder base. Thereafter, the binder is hardened and a composition is obtained consisting of a hardened binder containing embedded therein parallelly oriented mica flakes. As explained above, it is important to continue the orienting influence—in the present case the influence of the electrostatic field—while the binder is being hardened, e. g. dried, so as to ensure proper parallel orientation of the flakes in the finished composition.

Instead of using an electrostatic field for the purposes of the present invention, I might also subject the semi-liquid binder—mica mixture to the influence of electrical high-frequency oscillations, e. g. supersonic oscillations which have also an orienting effect upon the mica particles movably embedded, e. g. floating, in the liquid or semi-liquid binder. Also in this case, it is of importance to continue action of the high-frequency oscillations during hardening of the binder base.

I have found that compression of a plastic or semi-plastic binder—mica mass in opposite directions, e. g. by rolling or in a press, resulting in flowing of the binder—mica mass normal to the direction of pressure, has also an orienting effect, namely the mica flakes are oriented by such pressure in direction of flow of the mass, i. e. normal to the direction of pressure. Thus, it is possible to obtain by this method sheets and plates containing mica flakes oriented parallelly to each other and to the faces of these sheets and plates.

Similar effects can be obtained by drawing the plastic binder containing the mica flakes; during this process, the flakes are oriented parallelly to the direction of drawing and thus after hardening are embedded in the hardened binder parallelly to each other.

Finally, it is also possible to parallelly orient the mica flakes by extruding the plastic binder—mica mixture in which case the flakes will be oriented parallelly to the direction of extrusion.

I wish to note that although I have described above various embodiments of my new process, I have found that best results are obtained by subjecting a liquid or semi-liquid binder—mica mixture to an orienting influence, preferably an electrostatic field, as described above.

It will be understood that each of the elements described above, or two or more together, may also find a useful application in other types of

insulating materials differing from the types described above.

While I have described the invention as embodied in micaceous insulating materials and processes of producing the same, I do not intend to be limited to the details shown, since various modifications and changes may be made without departing in any way from the spirit of my invention.

Without further analysis, the foregoing will so fully reveal the gist of my invention that others can, by applying current knowledge, readily adapt it for various applications without omitting features that, from the standpoint of prior art, fairly constitute essential characteristics of the generic or specific aspects of this invention, and therefore such adaptations should and are intended to be comprehended within the meaning and range of equivalence of the following claim.

What I claim as new and desire to secure by Letters Patent is:

In the process of forming an insulating material of the character described, the steps of preparing an at least semi-liquid mixture of a hardenable electrically non-conductive binder and minute mica flakes floating therein, exposing said semi-liquid binder—mica mixture to an electrostatic field adapted to parallelly orient said minute mica flakes in said semi-liquid hardenable electrically non-conductive binder, and hardening said semi-liquid hardenable electrically non-conductive binder while said binder—mica mixture is still exposed to said electrostatic field, thus obtaining an insulating material consisting of a hardened electrically non-conductive binder and parallelly oriented minute mica flakes embedded therein.

EZEKIEL J. JACOB.

#### REFERENCES CITED

The following references are of record in the file of this patent:

#### UNITED STATES PATENTS

| 45 | Number    | Name    | Date           |
|----|-----------|---------|----------------|
|    | 389,519   | Lee     | Sept. 11, 1888 |
|    | 2,286,569 | Pollack | June 16, 1942  |
|    | 2,384,541 | Fruth   | Sept. 11, 1945 |

#### FOREIGN PATENTS

| 50 | Number  | Country       | Date        |
|----|---------|---------------|-------------|
|    | 2,287   | Great Britain | 1900        |
|    | 553,104 | Great Britain | May 7, 1943 |